

Patented Apr. 6, 1926.

1,579,435

## UNITED STATES PATENT OFFICE.

BRICE L. CLUTIER, OF CHICAGO, ILLINOIS, ASSIGNOR TO LIGHTNING PRODUCTS CORPORATION, A CORPORATION OF ILLINOIS.

### METAL CLEANER AND POLISHER.

No Drawing.

Application filed July 26, 1922. Serial No. 577,743.

*To all whom it may concern:*

Be it known that I, BRICE L. CLUTIER, a citizen of the United States, residing at Chicago, in the county of Cook and State 5 of Illinois, have invented certain new and useful Improvements in Metal Cleaners and Polishers, of which the following is a specification.

This invention relates to metal cleaners 10 and polishers.

One of the objects of the invention is to provide an improved metal cleaner and polisher.

Another object is to provide a cleaner and 15 polisher which is efficient and will not scratch nor mar or otherwise injure highly finished metal surfaces.

Another object is to provide a cleaner and polisher which will not injure the person 20 of the user or the surfaces of woods, paints and varnishes with which it may come in contact.

Another object is to provide a cleaner and polisher which is ready for instant use and 25 does not require an extraneous applicator.

Another object is to provide an impregnated cloth for use in cleaning and polishing metals.

Other objects and advantages will here- 30 inafter appear.

An embodiment of the invention is set forth in the following description.

The cleaning and polishing compound 35 comprises a mixture of silica, petrolatum and stearic acid. These ingredients are heated and mixed together.

The cleaning and polishing cloth is produced by impregnating a suitable textile with the compound.

The following proportions of ingredients 40 and procedure have been found to give excellent results.

To produce about seventy (70) pounds of the compound approximately twenty-five (25) pounds of water-floated, 350 mesh 45 hard silica, approximately thirty (30) pounds of amber petrolatum and about fifteen (15) pounds of stearic acid are placed together in a pot and heated to a freely fluid mixture. It is a good plan to agitate the 50 mixture to keep the silica evenly distributed through the compound.

This amount of compound is sufficient to properly impregnate about thirty (30) pounds of heavy grade cotton flannel. The 55 sheet of cotton flannel is immersed in the fluid compound and, after being thoroughly impregnated, is divested of any excess compound by being passed through rolls or other suitable means.

The cloth is then ready for use in polishing and cleaning metals. It appears to be practically dry and will retain its properties until substantially worn out.

Having described my invention, what I 65 claim as new and desire to secure by Letters Patent, is:-

A metal cleaning and polishing compound 70 consisting of the following ingredients in approximately the following proportions by weight twenty-five parts of hard silica, thirty parts of petrolatum and fifteen parts of stearic acid.

In testimony whereof I hereunto subscribed my name.

BRICE L. CLUTIER.